

March 2, 1926.

1,575,468

J. D. VOSS

EMBROIDERY

Filed August 7, 1925



Fig. 1.

Fig. 2.

Fig. 3.

Fig. 4.



Fig. 5.



Fig. 6.



Witness:

W. R. Clark

Invention:

By Jacob D. Voss  
Jones, Aldington, Ames & Seibert  
Attys.

Patented Mar. 2, 1926.

1,575,468

# UNITED STATES PATENT OFFICE.

JACOB D. VOSS, OF CHICAGO, ILLINOIS, ASSIGNOR OF FORTY ONE-HUNDREDTHS TO SERGE WRY, OF CHICAGO, ILLINOIS.

## EMBROIDERY.

Application filed August 7, 1925. Serial No. 48,696.

To all whom it may concern:

Be it known that I, JACOB D. Voss, formerly a resident of Russia and a subject of the Czar of Russia, not now a citizen of any country, residing at Chicago, in the county of Cook and State of Illinois, have invented new and useful Improvements in Embroidery, of which the following is a full, clear, concise, and exact description, reference being had to the accompanying drawing, forming a part of this specification.

My invention relates to embroidery.

One of the objects of my invention is to provide a beaded embroidery which will be artistic in appearance and which will be flexible and water proof, so that it will be durable and can be readily cleaned.

A further object of my invention is to provide an improved method of making such embroidery.

A further object of my invention is to provide an improved flexible water proof foundation of adhesive material to which the glass beads are applied.

Further objects will appear from the description and claims.

In the drawing in which my invention is illustrated, Fig. 1 is a face view of a piece of fabric showing the first step of applying the embroidery;

Fig. 2 shows the second step;

Fig. 3 shows the third step;

Fig. 4 is a section on the line 4—4 of Fig. 1;

Fig. 5 is a section on the line 5—5 of Fig. 2;

Fig. 6 is a section on the line 6—6 of Fig. 3; and

Fig. 7 is a face view showing a design somewhat different from that shown in Figs. 1, 2 and 3.

Referring first to Figs. 1 to 6, inclusive, the first step in the method is to outline the figure as shown in Fig. 1. This may be done by the use of a paste filled tube. The paste, the composition of which will be described hereinafter, may be squeezed from this tube in the form of thread or ribbon 1, the tube being moved along above the surface of the cloth or other fabric 2 to cause the ribbon as squeezed from the tube to outline the pattern which is to be filled in afterward. Previous to the applica-

tion of the ribbon of paste, the outline of the pattern may be indicated on the fabric in any suitable manner as by the use of powdered material applied through a perforated stencil.

While this paste ribbon outline is still sticky, an ornamental coating of any desired material, such as bronze powder, may be dusted over the pattern. A coat of this bronze dust will adhere to the sticky ribbon. The pattern thus outlined is allowed to dry for a sufficient time to allow the paste ribbon to harden and become non-adhesive, after which any of the bronze dust which has not adhered to the paste ribbon may be brushed off.

The next step in the process, as shown in Fig. 2, is to fill in inside of the hardened ribbon outline with a suitable foundation material 3 (which material may be the same as the material used in the ribbon). This filled in foundation may be applied by squeezing the paste from a tube and spreading it out by means of a brush. It is preferable to leave a slight space between the outer edge of this filled in foundation and the ribbon outline as shown at 4 in Figs. 5 and 6. As soon as this filled in foundation is completed, while it is still sticky, it may be colored in any suitable manner and design as by the application of oil paint to give the desired color effect. The layer of glass beads 5 is then applied as indicated in Fig. 3 while the filled in foundation is still sticky. These beads may be applied simply by covering the design with a pile of the beads and shifting this pile around until all parts of the pattern have been covered. The pile of beads may be shifted around simply by lifting up first on one part of the fabric and then another until all parts of the pattern are covered with a layer of the beads, as shown in Figs. 3 and 6.

I have discovered that a foundation material suitable for the purpose is obtained by mixing together oil, paint powder, and rubber cement in approximately the proportions of one part oil, three parts rubber cement and six parts paint powder, these proportions being by weight. I first mix together the oil and paint powder, and then mix the combined oil and paint powder with the rubber cement. This foundation results

in a beaded embroidery which is flexible and water proof so that the beads do not crack off and so that the embroidery may be cleaned. Almost any cleaning liquid may be used except turpentine without injuring the material in any way.

The embroidery shown in Fig. 7 makes use of the same general method as described above but in this form the filled in foundation is in the form of small points or dots 6 and lines 7, and the color effect is obtained by the use of different colors of beads instead of by applying different colors of paint to the foundation. In this form the outline of paste ribbon is applied just as in the form previously described. The foundation within the outline is then filled in, a section at a time. If a certain part of the pattern is to be covered with, for instance, blue beads, the dots or points of pasty foundation are applied to that portion of the pattern and the glass beads are applied to the part of pattern thus covered, just as in the form previously described. The artist then applies the points or dots of the sticky foundation to another portion of the pattern which it may be desired to have covered with beads of another color and the beads of the desired color are then shifted around over the surface of the pattern, but they do not stick to the portion of the pattern which has been previously covered with the beads of another color, but stick only to the uncovered points or dots of the sticky foundation material. In this manner beads of any

desired color may be applied to any desired portion of the design.

I claim:

1. The art of making beaded embroidery on fabrics comprising applying a ribbon of adhesive material to outline the design, covering the ribbon outline with powdered coloring material, allowing the ribbon outline to dry, filling in the space within the outline with a plastic adhesive foundation material, applying a colored surface coating to the foundation, and applying a layer of glass beads to the adhesive foundation.

2. The combination with a flexible fabric of a flexible water proof beaded embroidery thereon, comprising a plastic adhesive foundation and a layer of beads applied thereto, said adhesive foundation comprising a mixture of rubber cement, oil, and powdered paint, said mixture comprising approximately 10% oil, 30% rubber cement and 60% powdered paint.

3. The combination with a flexible fabric of a beaded embroidery thereon comprising a ribbon of adhesive material to outline the design, the ribbon outline being covered with powdered coloring material, a plastic adhesive foundation filling in the space within said outline and provided with a colored surface coating and a layer of glass beads applied to the adhesive foundation.

In witness whereof, I have hereunto subscribed my name.

JACOB D. VOSS.